

## UNITED STATES PATENT OFFICE

WILFORD J. HAWKINS, OF CLAIBORNE, MARYLAND, ASSIGNOR TO AMERICAN MACHINE & FOUNDRY COMPANY, A CORPORATION OF NEW JERSEY

## METAL FOIL

No Drawing.

Application filed May 16, 1928. Serial No. 278,346.

This invention relates to metal foil primarily designed to be used in place of tin foil.

Tin foil is in common use for wrapping articles. It can be rolled to a thinness of .001" without breakage, but it lacks sufficient malleability to enable it to be rolled any thinner than that.

It has now been discovered that lead containing from  $\frac{1}{4}$  to  $\frac{1}{2}$  of 1% of magnesium possesses sufficient malleability to enable the metal to be rolled into metal foil of a thinness of less than .0005", because the malleability of both metals used exceeds that of tin, or that of the lead-tin alloy commonly used in making tin foil. In practice, the new alloy is rolled to a thinness of .00045".

In making the new foil, the lead is first melted, and thereafter the magnesium is introduced into the molten lead by immersion. If the quantity of magnesium so introduced is all, or less than all, the lead will absorb, all of it will be absorbed. If, however, too much magnesium is introduced, approximately  $\frac{1}{2}$  of 1% will be absorbed and the excess will be wasted.

The new foil may be used alone as wrapping material, or as a facing for paper wrapping material, as tin foil may be used.

By the use of the new alloy in the form of metal foil of extreme thinness, a material saving in weight is effected; and since the metals used are cheaper than tin, a further material saving in cost is effected. Furthermore, the addition of the silver-bright magnesium to the lead makes the resultant alloy brighter in color than the lead-tin alloy commonly used in making tin foil; and the new foil of less than .0005" thinness is as strong as the old tin foil, which is more than twice as thick.

What is claimed is:

1. Metal foil composed of lead containing from  $\frac{1}{4}$  to  $\frac{1}{2}$  of 1% of magnesium and rolled to a thinness of approximately .0005".

2. Wrapping material comprising paper, and a facing of metal foil composed of lead containing from  $\frac{1}{4}$  to  $\frac{1}{2}$  of 1% of magnesium and rolled to a thinness of approximately .0005".

In testimony whereof, I have signed my name to this specification.

WILFORD J. HAWKINS.

55

60

65

70

75

80

85

90